

Dec. 18, 1962

P. E. QUENEAU ET AL  
AUTogenous PYROMETALLURGICAL PRODUCTION  
OF NICKEL FROM SULFIDE ORES

3,069,254

Filed Aug. 23, 1960

2 Sheets-Sheet 1



PAUL E. QUENEAU  
LOUIS S. RENZONI  
INVENTOR.

BY *C. Dr. Waller*

ATTORNEY

Dec. 18, 1962

P. E. QUENEAU ET AL  
AUTogenous PYROMETALLURGICAL PRODUCTION  
OF NICKEL FROM SULFIDE ORES

3,069,254

Filed Aug. 23, 1960

2 Sheets-Sheet 2



FIG. 3

PAUL E. QUENEAU  
LOUIS S. RENZONI  
INVENTOR.

BY *G. Dr. Deller*

ATTORNEY

1

3,069,254

## AUTOGENOUS PYROMETALLURGICAL PRODUCTION OF NICKEL FROM SULFIDE ORES

Paul Etienne Queneau, Fairfield, Conn., and Louis Scondo Renzoni, Copper Cliff, Ontario, Canada, assignors to The International Nickel Company, Inc., New York, N.Y., a corporation of Delaware

Filed Aug. 23, 1960, Ser. No. 51,438

12 Claims. (Cl. 75—82)

The present invention relates to an improved process for the smelting and refining of nickel- and copper-containing sulfide materials for the direct recovery of metallic nickel or nickel-copper alloys therefrom.

Attempts have been made in the past to produce metallic nickel directly from nickel-containing matte. Thermodynamically and kinetically the reactions between nickel sulfide, oxygen and nickel oxide in a converter allow full conversion of nickel matte to metallic nickel. Although entirely feasible theoretically, an operable process based on these reactions has not heretofore been developed.

Borchers was perhaps the first to attempt to blow nickel matte to metal employing an oxygen blast, but because of lack of temperature control and improper gas-liquid-solid contact he was unsuccessful. We are familiar with the pioneer work of Lellep on the desulfurizing of nickel matte and nickel-copper matte to metallic nickel and nickel-copper alloys, respectively, by blowing in a converter. Lellep considered surface blowing in an effort to solve the insuperable problems which he encountered when employing submerged tuyères at the high temperatures he was attempting to use. Lellep did not appreciate, however, the absolute necessity for efficient gas-solid-liquid contact essential for bath uniformity and achievement of equilibrium between the several reactants and the overriding advantages of using oxygen or oxygenated air. Instead he neglected the advantages which are derived from mechanically induced bath turbulence and he resorted to preheated air or to extraneous heat from oil, coal or electric energy, and finally relied upon the standard Bessemer steel converter for attempted application of his process. Following the failure of Lellep, Shoffstall et al. did further work on improving the bessemerizing of nickel-containing mattes to desulfurize such mattes. They attempted to accomplish this by forcing super-heated steam through the molten matte employing submerged tuyères but their process was impractical. Shoffstall et al. also failed to recognize the necessity of proper gas-liquid-solid contact and of the advantages of using a gas rich in oxygen relative to air.

The Bessemer converter is employed in the copper industry to convert copper sulfide to metallic copper. In converting nickel-bearing iron sulfide in the molten state to low iron-nickel sulfide, the art also depends on the use of the Bessemer concept involving an air blast below the molten matte level through tuyères. However, it is impossible to blow nickel sulfide to metallic nickel in this manner. For this purpose the air must be highly preheated or oxygenated or fuel must be added to maintain the required reaction temperatures. However, such modification of the Bessemer principle is impractical because of resulting excessive localized temperature rise and refractory attack, inadequate gas-solid-liquid contact with resulting non-uniformity of the bath, massive, localized nickel oxide accumulations and inadequate control of operating variables.

Although Lellep, Shoffstall and others made attempts to overcome these and other difficulties, they were unable to develop a commercially operable process.

We have now discovered that sulfide materials rich in nickel, such as ores, concentrates and mattes, may, after

2

preliminary preparation, if necessary, be successfully converted autogenously and directly to metallic nickel by the use of an oxygen-rich stream directed onto these materials at least a portion of which are in the molten state while providing efficient and effective gas-liquid-solid contact throughout the bath, i.e., by induced turbulence and controlling oxygen supply and temperature. Furthermore, another critical deficiency in the prior art which prevented continuous liquid phase production of metallic nickel was the inability to remove the copper which is normally associated with the sulfide ores of nickel. We have also discovered that such copper may be continuously separated from nickel by a major improvement in the obsolete and abandoned Orford process.

It is an object of the present invention to provide a process for the autogenous pyrometallurgical production of nickel or nickel-copper alloys from nickel-copper sulfide mattes.

Another object of the invention is to provide a method for producing metallic nickel directly from nickel-rich sulfide materials such as mattes by inducing turbulence of the liquid material and by impinging process gases on the physically and chemically active surface thereof.

The invention also contemplates providing a novel process for the direct reduction of substantially iron-free nickel mattes to nickel metal anodes.

The invention further contemplates providing novel methods for separating copper and cobalt from low iron-nickel mattes and for reducing the nickel sulfide directly to metallic nickel.

It is a further object of the invention to provide an autogenous method for eliminating rock, iron and sulfur from nickel-rich sulfide concentrates such as pentlandite concentrates and obtaining nickel metal low in copper, cobalt and precious metals and a sulfur dioxide-rich gas suitable for economic sulfur fixation.

Other objects and advantages will become apparent from the following description taken in conjunction with the accompanying drawing in which:

FIGURE 1 shows a longitudinal section through a rotary kiln-type furnace in which the autogenous smelting and desulfurizing of nickel-rich sulfide materials to metallic nickel according to the herein-described process may be carried out;

FIG. 2, depicts a cross-section of the same furnace through line 2—2 of FIG. 1; and

FIG. 3 shows a diagrammatic cross-section through a liquid-liquid extraction column in which copper may be separated from nickel sulfides by the special solvent extraction process described hereinafter.

According to the present invention, nickel-containing sulfide materials such as nickel matte and crude nickel sulfide precipitates such as those obtained by ore leaching techniques are smelted autogenously in a rotary kiln-type furnace to a matte. This is followed by top-blowing the matte so obtained in the same autogenous, rotary kiln-type furnace using commercial oxygen or oxygen-enriched air directed down onto the surface of the molten bath but not through the metal from below the liquid level. By proper control of oxygen supply and bath temperature and by strong mechanically-induced agitation of the bath the molten nickel sulfide is reduced to substantially sulfur-free nickel metal. The blowing and mechanical agitation of the bath are controlled each independent of the other. Control of oxygen supply and of turbulence is such as to maintain satisfactory bath fluidity and uniformity to permit rapid nickel sulfide-nickel oxide reaction and high efficiency of oxygen utilization while maintaining the temperature below that at which undue refractory attack is experienced. When the sulfur content has been decreased to less than about 4% and at which time sufficient oxygen is normally present

in the bath to oxidize this sulfur, the blast is replaced by oxygen-impoverished gases, i.e., gases having an oxygen content insufficient to cause visible formation of interfering amounts of nickel oxide dross on the surface of the agitated bath. It is critically important that such gases be at such a high temperature as to permit bath temperature regulation in the 3000° F. to 3200° F. range. At the same time, strong mechanically-induced agitation is continued or increased in intensity to maintain efficient and effective gas-solid-liquid contact throughout the bath. The turbulence in the bath is mandatory to insure bath uniformity, both physical and chemical, so as to give quick reaction towards equilibrium, e.g., the nickel oxide-nickel sulfide reaction. By this technique sulfur in the molten bath may be eliminated to less than about 0.05% sulfur, e.g., 0.01% sulfur. It will be understood of course, that alternatively standard desulfurization techniques can be employed for final sulfur removal.

Agitation of the bath to insure adequate gas-liquid-solid contact is obtained by rotating the furnace and by blowing the oxygen-rich gas stream onto the turbulent molten bath from above the liquid level. It has been found that the blowing operation may be conducted initially at temperatures not greatly above the melting point of the nickel sulfide-containing material and at this stage advantage is taken of the exothermic heat of reaction to smelt solid feed if desired. However, it is preferred to heat the nickel sulfide to a temperature of at least about 2400° F., avoiding formation of surface oxide, under weakly or non-oxidizing conditions prior to blowing with commercial oxygen. If no melting is to take place and molten matte at elevated temperature is available, proper rate and degree of heating can be achieved by control of oxygen addition. The temperature is raised as desulfurization proceeds until, at a sulfur content of the bath of less than 4%, advantageously between about 1% and about 3%, a temperature between about 3000° F., and 3200° F., is attained and maintained until final sulphur elimination is achieved. It will be understood that if the nickel contains a substantial proportion of copper, final temperatures will be significantly lower.

In carrying one embodiment of the invention into practice, nickel matte, which may contain less than about 1% iron, the amount of copper remaining after conventional separation of copper by ore dressing means, e.g., one part of copper to ten parts of nickel, and some cobalt and precious metals, e.g., one part of cobalt to 25 parts of nickel and 2 ounces of precious metals per ton of nickel, is treated, if desired, for the removal of the copper, cobalt and precious metals as hereinafter described. The matte is then transferred to the autogenous reduction furnace wherein it is top blown with oxygen to nickel metal.

The autogenous reduction operation may be carried out in the furnace depicted in FIG. 1 and FIG. 2 of the accompanying drawing which show a longitudinal section of the furnace and a cross-section of the furnace through line 2-2 of FIG. 1, respectively. Referring to FIGS. 1 and 2, the molten, nickel sulfide-containing material 10 is treated in a rotary kiln-type furnace 11 which is lined with high-grade refractory brick 12. The furnace may be tilted as desired for tapping by using tilting mechanism 20. The furnace has tires or drive rims 13 affixed circumferentially around it and these tires rest on supporting or drive wheels 14. Oxygen or oxygen-enriched air is supplied by a water-cooled tube or pipe 15 which projects through seal 21 and opening 16 into the furnace. Exhaust gases pass out of opening 17 at the other end of the furnace into the flue 18 which may be water-cooled and which may be swung away from the kiln opening to allow charging of fresh sulfide, flux or other materials through opening 17. Solids may be alternatively charged through opening 16 upon removal of pipe 15 and seal 21. Seal 22 provides a gas-tight contact between the kiln and flue 18. Slag may be withdrawn by tilting the furnace and tapping from the top of the molten bath. At the com-

pletion of the blow, molten metallic nickel is tapped by tilting the furnace into the position shown by 23 in FIG. 1 or is optionally withdrawn through taphole 19.

The reduction operation need not be conducted in the apparatus as specifically shown in FIG. 1 and described hereinbefore providing the apparatus meets the operational requirements as outlined herein, e.g., it may be carried out in a top blown converter such as the Kaldo furnace.

10 Based on tonnage tests, which we have conducted, we estimate that a single furnace of the above-described design, with effective inside diameter of about 17 feet, can produce commercial nickel at the rate of about 500 tons per day.

15 Nickel matte which is substantially iron-free may be blown directly to metallic nickel after copper removal, if necessary, from the molten material as described hereinafter. Precious metals may be removed as described hereinafter before blowing directly to metallic nickel.

20 The sulfide material which has been charged into the furnace is treated by bringing oxygen or oxygen-enriched air into direct contact with its surface. This gas, which advantageously is initially commercial oxygen, is blown into the furnace above the surface of the molten material.

25 Necessary bath turbulence is maintained by continuous rotation of the furnace at a substantial speed.

30 In the first stage of the blow the temperature of the bath is kept high enough to keep the reacting materials in a sufficiently fluid state to permit rapid reaction and yet below the temperature at which undue refractory

35 penetration or erosion is experienced. For relatively pure nickel matte which melts at about 1450° F., the furnace blow may be started at a temperature of as low as 1550° F. However, in most circumstances it is preferred to initiate the blow with commercial oxygen at much higher temperatures than 1550° F., e.g., 2500° F., in order to avoid formation of nickel oxide slag and accretions. For sulfides containing substantial amounts of iron as well as nickel, such as pentlandite concentrate, and which require considerable slagging off of iron, the temperature must be high enough to keep the slag in a fluid state.

40 It is important that substantially all iron is eliminated and any slag is removed from the furnace before blowing for sulfur removal to form metallic nickel is commenced. It has been found that any formation of slag during reduction of the nickel matte to metallic nickel results in serious decrease in gas-liquid contact and lowers oxygen efficiency. Thus, only by keeping the surface of the molten bath reasonably clear of slag is economic desulfurization in the autogenous reduction furnace possible.

45 As sulfur elimination of the bath by the top blowing with oxygen or oxygen-enriched air proceeds, the temperature of the bath is rapidly raised until the sulfur content of the bath has been lowered to preferably between about 1% and about 3% and a bath temperature of more than about 2800° F. has been attained. It has been found that the temperature of the reduction operation and, in fact, the operation in general is controlled by varying the oxygen supply, by observing exhaust gas analysis and temperature and by varying turbulence.

50 During this first stage of sulfur elimination down to between about 1% and about 3% sulfur, it is preferable to inject as much oxygen as is practicable without causing undue nickel oxide slag formation or too much splash formation at the mouth of the furnace. Use of

55 commercial oxygen allows more rapid nickel reduction and production of gas rich in sulfur dioxide, e.g., 75% sulfur dioxide, but excess heat is also thereby generated. Part of this heat is utilized for heating the charge to the temperature desired for final sulfur elimination, i.e., between about 3000° F. and 3200° F. It may be desirable to cool by injecting air into the furnace. The addition of air may be, of course, undesirable in lowering the sulfur dioxide content in the exhaust gas and increasing the gas quantity required per unit volume of injected oxygen.

Cooling may be otherwise accomplished or may be supplemented by adding water to the gas stream rather than air or by adding solid charge to the furnace or by a combination of these techniques.

When desulfurization has proceeded to preferably between about 1% and about 3% sulfur, e.g., 2% sulfur, the oxidizing gases should be replaced, as aforementioned, by substantially sulfur-free oxygen-impoverished gases, e.g., neutral or somewhat reducing gases while heating or maintaining the molten bath to a temperature of between about 3000° F. and about 3200° F. To maintain this temperature in the bath, the neutral or reducing gases must be at a high temperature and this is best accomplished by adding a highly combustible fuel such as natural gas or propane together with the oxygen. The fuel consumes any excess oxygen and generates a high temperature flame so that undue formation of nickel oxide is thereby prevented. The impinging gases may thus advantageously and gradually be decreased in oxygen content from that of commercial oxygen, to oxygen-enriched air, to air, to oxygen-impoverishment, to non-oxidizing or inert and finally to somewhat reducing. It will be understood that once adequate oxygen supply is present in the bath, the function of the impinging gases is heat supply and insurance of a low sulfur dioxide partial pressure atmosphere. The exact oxygen content of the gas is a variable determined by and within the control of the furnace operator. It has been found that during this final desulfurization period best results are obtained by increasing bath turbulence especially if for any reason the bath has become over-oxidized.

By the above novel technique, desulfurization of the molten nickel proceeds to less than 0.05% sulfur, e.g., 0.01% sulfur. Blowing of molten nickel sulfide material down to these low sulfur contents on a tonnage basis has been found to be attainable in less than 8 hours.

Final desulfurization, which is carried out under a neutral or somewhat reducing atmosphere, is essentially achieved by reaction between residual sulfur and oxygen in the molten metal. A surprisingly high absorption of oxygen takes place in our metal bath before any visible oxide film on its surface appears. Thus, in one case, an apparent dissolved oxygen content of 9.5% was obtained while the metal was at a temperature of 3100° F., which is a much higher content than expected from study of the nickel-oxygen equilibrium diagram. We believe a substantial proportion of this oxygen was present as an extremely finely-divided, uniformly dispersed, solid nickel oxide phase. High oxygen content in the sulfur-bearing bath is a key feature of our turbulent metal desulfurizing process in that it permits elimination of the oxidizing furnace atmosphere at a much higher sulfur content of the metal bath than in the prior art. The oxygen content of the bath required for effective final desulfurization, of course, need not be as high as the above. Sulfur is preferably eliminated without forming visible oxide floating on the surface, i.e., temperature and oxygen addition is so controlled as to maintain a shiny surface on the metal bath. Speed of refining increases the higher the oxygen content of the bath without surface oxide formation, e.g., without substantial clouding of the bath surface.

As stated hereinbefore, the surface of the molten bath should be kept free of slag or scum. For this purpose the oxidizing gases in the furnace preferably should be replaced by non-oxidizing gases before sulfur elimination has proceeded to below about 1% sulfur, e.g., 2% sulfur. Deoxidation of the molten bath after sulfur removal may be readily carried out by carbon addition to the furnace. Graphite has been found to be an excellent deoxidizing agent although other deoxidants such as silicon or aluminum may be utilized. A high residual oxygen content in the bath should, of course, be avoided since large quantities of costly deoxidizing agents are required and possibly violent reactions may occur.

In a modified procedure for carrying out the reduction

of nickel sulfide to metallic nickel by our novel techniques the final desulfurization from below 4% sulfur is carried out in a separate furnace in the same manner as described hereinbefore. This modified procedure may be advantageous over doing the complete operation in one furnace. Thus, final refining may be carried out in a furnace the walls of which are not impregnated with sulfide which has the effect of delaying the lowering of sulfur content in the bath and also presents a risk of re-absorption, if deoxidation is carried out inside the furnace before tapping. There is a further advantage in using a second furnace in that brick which is not impregnated with sulfide will allow increased refractory strength at the high temperature necessary during final desulfurization. Furthermore, the two furnace technique will allow steady operation in one furnace which is utilizing oxygen only and so attain an even production of gas with a high sulfur dioxide content produced while using the second furnace which is utilizing oxygen-impoverished gases with generally more rapid furnace rotation. Also, any oxide formed in the first furnace could be easily retained therein for subsequent reaction with green charge, with the final blow in the second furnace being carried out without risk of slag formation.

It is to be noted that the herein described novel reduction of nickel sulfide to metallic nickel can be attained with very small nickel losses due either to slagging as oxide or to dusting in exhaust gases, i.e., a nickel yield in excess of 99%. We have produced nickel by our process on a tonnage basis containing 0.009% sulfur, 0.02% silicon, 0.0017% lead, 0.0001% zinc, 0.0004% bismuth and 0.0014% antimony.

The extreme importance and necessity connected with strong induced turbulence of the furnace bath, as described hereinbefore, is demonstrated by the failure to obtain the desired results by blowing in a stationary furnace as shown in Example VII described hereinafter in which the nickel reduction reaction ceased at a sulfur content of 2% in the bath due to excessive local oxidation and resultant formation of a floating impenetrable, hard, nickel oxide blanket. A similar result is obtained if attempts are made to reduce the sulfur content of the bath to below about 1% sulfur before replacing the oxygen with high temperature, weakly oxidizing, non-oxidizing, neutral and/or reducing gases which we have termed oxygen-impoverished gases and which have an oxygen content insufficient to cause visible formation of interfering amounts of nickel oxide dross on the surface of the agitated bath; e.g., with a free oxygen content of less than about 3%. In cases where iron-containing nickel matte is first blown in the autogenous reduction furnace for iron removal, the slag formed is treated for recovery of its nickel content. Advantageously, slag produced during the first stage of iron elimination which is low in nickel is removed and treated for recovery of its nickel content, if desired, and the slag produced during the final stage of iron elimination is left in the furnace for recovery of its nickel content upon further addition of concentrate or matte. After a complete charge of molten matte has been built up in the autogenous furnace, slag produced from final iron elimination is removed and may be treated in parallel autogenous reduction furnace for treatment with fresh sulfide.

In the instances where nickel sulfide materials to be treated by this process contain amounts of copper or cobalt which may not be acceptable in the nickel metal, e.g., more than about 0.10% copper and/or more than about 0.75% cobalt in the metal, the sulfide material must be processed for their removal.

The copper advantageously should be removed before desulfurizing treatment in the top blown reduction furnace. Copper removal by means of a novel solvent extraction process, i.e., high temperature liquid-liquid

extraction, has been found particularly advantageous. By this technique we have found that nickel sulfide with a substantial copper content, e.g., a ratio of nickel:copper of, for instance, 10:1 can be treated for copper removal to produce a nickel sulfide having a residual copper content of less than 0.10%, e.g., with a ratio of nickel:copper of at least about 1000:1. As a general rule nickel sulfide ores containing copper can be concentrated by flotation so that the bulk of the nickel is in a concentrate containing nickel and copper in a ratio of at least about 10:1 which can be readily decopperized by our novel procedure. Much higher copper contents can be extracted by this method if simpler prior separation, e.g., of the natural minerals by flotation, is impractical.

This novel molten salt solvent extraction technique is based on the use of sodium sulfide as the selective agent, probably a complexing agent, for copper sulfide. This agent is dissolved in molten sodium chloride in which solution nickel has only a slight solubility and copper a high solubility. An essential feature of this salt combination is its relatively low melting point of below about 1300° F. This permits the solvent extraction to proceed at a temperature as low as about 1350° F. Thus, the extraction is carried out close to the melting point of the metal sulfides which is the optimum temperature for liquid copper-nickel separation. This low operating temperature and the high water solubility of the extractant have the additional important advantages of economy in reagent, fuel and refractories consumption.

This novel separation technique is outstanding in that sequestration of copper by the solvent and isolation of nickel are both highly effective while the cost of labor, supplies and equipment is relatively low. Our procedure permits economical removal of copper sulfide, entirely beyond the capability of the existing art, from sulfides having a broad range of nickel to copper ratios to yield nickel sulfide having a nickel to copper ratio of greater than 1000:1.

The highly beneficial effect of using a solvent, such as sodium chloride for sodium sulfide is clearly demonstrated by the following example:

#### EXAMPLE I

150 grams of matte, containing 68.2% nickel and 3.25% copper, was mixed with 150 grams of sodium sulfide and the mixture was melted at 1550° F. The upper sodium-rich and the lower nickel-rich fractions were tapped from the bottom of the crucible into separate containers although there was found to be no sharp physical definition between them. Analyses of these upper and lower layers gave the results as shown in Table I.

Table I

|                            | Weight, percent | Analysis   |            | Ni:Cu Ratio | Percent of Total Nickel |
|----------------------------|-----------------|------------|------------|-------------|-------------------------|
|                            |                 | Percent Cu | Percent Ni |             |                         |
| Upper Sodium-Rich Fraction | 49.4            | 1.7        | 30.0       | 18:1        | 43.5                    |
| Lower Nickel-Rich Fraction | 50.6            | 1.4        | 38.0       | 27:1        | 56.5                    |

The test was then repeated except that 75 grams of sodium chloride and 75 grams of sodium sulfide were used instead of 150 grams of sodium sulfide. Two distinct liquid fractions were obtained by this test which were cleanly separated by bottom tapping. The two fractions were then analyzed to give the results as shown in Table II.

8  
Table II

| 5                          | Weight, percent | Analysis   |            | Ni:Cu Ratio | Percent of Total Nickel |
|----------------------------|-----------------|------------|------------|-------------|-------------------------|
|                            |                 | Percent Cu | Percent Ni |             |                         |
| Upper Sodium-Rich Fraction | 46.4            | 2.7        | 4.9        | 2:1         | 6.2                     |
| Lower Nickel-Rich Fraction | 53.6            | 0.4        | 64.4       | 100:1       | 93.8                    |

In this novel liquid-liquid solvent extraction technique about one-half to double by weight of a mixture of sodium chloride and sodium sulfide may be melted with the copper-containing nickel sulfide material. The sodium chloride-sodium sulfide mixture advantageously may contain between about 25% and about 75% sodium chloride. It will be understood that although we prefer sodium chloride, other chloride modifiers such as the chlorides of potassium, calcium and aluminum may be employed. The nickel sulfide material and sodium salts are advantageously melted at not below about 1350° F. and not above about 1550° F., carefully mixed to insure excellent countercurrent liquid-liquid contact and then separated by gravity into copper-rich and nickel-rich fractions. A preferred apparatus for this purpose is a liquid-liquid extraction column as shown in FIGURE 3. The substantially copper-free nickel sulfide product may be air blown for slagging of residual sodium salts and then transferred directly to the autogenous reduction furnace to be blown to metallic nickel as described hereinbefore. The copper-sodium rich product may be treated by water leaching to recover copper and the sodium salts and residual nickel. Alternatively, the extraction may be carried out in other apparatus, e.g., in an appropriately designed, countercurrently operated rotating kiln or by simple ladle mixing, settling and bottom pouring in a countercurrent multi-stage operation. The advantageous results obtained by our novel solvent extraction technique for extracting copper from nickel sulfide are shown in Examples II and III.

#### EXAMPLE II

A nickel matte containing 3.25% copper with the balance mainly nickel and sulfur, was treated for copper extraction by a multi-stage countercurrent liquid-liquid extraction at 1550° F. The solvent, 50% by weight of sodium sulfide and 50% by weight of sodium chloride, was added to an equal weight of nickel matte in a crucible, mixed thoroughly and the nickel sulfide was tapped from the bottom at each of four extraction stages. Salt fraction was mixed with the appropriate nickel sulfide bottoms in each of these stages. The final products from the four-stage treatment analyzed as follows:

| 60 |                           | Analysis, Percent |      | Ni:Cu Ratio |
|----|---------------------------|-------------------|------|-------------|
|    |                           | Cu                | Ni   |             |
| 65 | Final Copper-Rich Solvent | 4.20              | 1.2  | 0.3:1       |
|    | Final Nickel Sulfide      | 0.03              | 63.3 | 2110:1      |

#### EXAMPLE III

A nickel matte containing 4.8% copper with the balance mainly nickel and sulfur was treated for copper extraction in the same way as in Example II except that the countercurrent extraction was conducted at 1400° F. The final products from the four-stage treatment analyzed as follows:

|                           | Analysis, Percent |      | Ni:Cu Ratio |
|---------------------------|-------------------|------|-------------|
|                           | Cu                | Ni   |             |
| Final Copper-Rich Solvent | 6.25              | 1.2  | 0.2:1       |
| Final Nickel Sulfide      | 0.06              | 63.3 | 1050:1      |

It has been found highly advantageous to use a continuous countercurrent solvent extraction technique to attain copper removal down to less than about 0.1% copper in the nickel sulfide material. The countercurrent liquid-liquid extraction may take place in a standard type of apparatus such as that shown in FIGURE 3 which depicts the diagrammatic cross-section of a baffle plate column in which the copper-containing nickel sulfide is treated with the molten salt mixture for elimination of copper. Referring to FIGURE 3, solid baffle plates 30, which extend partially across the column cross-section, are placed at suitable intervals in the column. Molten copper-containing nickel sulfide from storage tank 31 is introduced through line 32 and variable orifice 33 into the top of the column at 34. Molten sodium salt solvent from storage tank 35 is introduced through line 36 and variable orifice 37 into the bottom of the column at 38. Nickel sulfide from which copper has been eliminated is drawn off the bottom of the column through line 39 and variable orifice 40. Copper-rich solvent is drawn off the top of the column through line 41. Heat is supplied to the column and to the tanks 31 and 35 to maintain the sulfide and sodium salts in a molten condition and at the separation temperature desired such as by way of electric immersion heaters 42 and external electric heaters 43.

The heavier nickel sulfide flows along each baffle, which is supplied with a short lip 44 so that each is substantially a tray, overflows over the lip and then flows downward to the next tray. The lighter sodium salt solvent flows upward around each baffle and through the free area between the tray and the inside walls of the column. Thus, as the sodium salt solvent rises through the falling nickel sulfide and removes copper sulfide, it becomes progressively richer in copper sulfide, while the nickel sulfide has more and more copper sulfide extracted as it flows downward.

A mini-plant multi-tray column of the above general design, 3 inches I.D. by 48 inches high was operated at a feed rate of up to one-half ton per day of copper-bearing nickel sulfide employing as a solvent a salt mixture consisting of sodium sulfide and sodium chloride and containing between 25% and 75% sodium chloride. In this simple device we were able to continuously lower the copper content of the nickel matte in a ratio of about 10:1, producing a nickel sulfide with a Ni:Cu ratio exceeding 1000:1 when treating mattes in the 0.75% Cu to 3.5% copper range. The test results indicated that nickel sulfide having a substantially higher copper content, e.g., 10% copper, could also be successfully treated.

Based on equilibrium data established for our novel liquid-liquid extraction system in the laboratory and further substantiated by the above mini-plant experiments, copper reductions by weight of 100:1 or more can be realized from cupriferous nickel sulfide when using our process in commercial extraction equipment such as tray columns, packed columns or mixer-settlers.

It is to be observed that our novel technique for removing copper from nickel mattes before blowing to metallic nickel permits a much higher degree of copper elimination therefrom than can be obtained by controlled cooling and flotation of the matte, i.e., less than 0.05% Cu as compared to more than 0.50% Cu.

As stated hereinbefore the molten nickel matte from which the copper has advantageously been extracted down to below about 0.10% copper may be transferred to the autogenous reduction furnace, preferably after residual

70 sodium salts have been removed by a brief, relatively low-temperature air blow in a separate vessel and decanted for reuse. However, in cases where there are precious metal values associated with the nickel sulfide material the precious metals may be removed by known means such as by blowing to create a sulfur deficiency, cooling, solidifying, grinding and removing the precious metals concentrated in the metallics. The nickel sulfide may then be water leached to remove sodium salts, dried and then fed directly to the autogenous reduction kiln.

10 In special circumstances, cobalt elimination may be accomplished during conversion of the sulfide material to metal by blowing the molten material with an oxygen-rich gas at a sulfur content of more than about 3% to selectively oxidize the cobalt in the presence of a flux such as silica. The cobalt is then skimmed off as slag. The sulfur content of the molten charge is maintained at above about 3% sulfur by continuously adding fresh sulfide material to the autogenous reduction furnace while top-blowing at between about 2300° F. and about 2800° F. for sulfur and cobalt removal. When the furnace has received a full charge and adequate cobalt removal has been achieved, the top-blowing of the molten charge is then completed as described hereinbefore to form metallic nickel. The cobalt-rich slag can be conveniently treated for cobalt recovery by known means. It will be understood, however, that formation of this slag can interfere with our process, as hereinbefore described, so that cobalt removal in this manner is not always practicable.

15 20 25 30

The following example illustrates the satisfactory results that may be obtained by our technique for eliminating cobalt from nickel sulfide:

#### EXAMPLE IV

35 Molten nickel matte containing 2.7% cobalt and the balance substantially nickel and sulfur was partially reduced to 10% sulfur at 2500° F. by top blowing with oxygen. Siliceous flux was then added and the oxygen blow was continued for 15 minutes to selectively oxidize cobalt and remove it as slag. The final low-sulfur matte contained 0.6% cobalt, 90.3% nickel and the balance mainly sulfur. The ratio of nickel to cobalt was increased by this treatment from 25:1 to 150:1.

40 45 For the purpose of giving those skilled in the art a better understanding of the invention, the following illustrative examples are given:

#### EXAMPLE V

50 A sulfide ore containing nickel, copper, cobalt, iron and gangue-minerals was treated by conventional methods to produce a concentrate containing 12.0% nickel, 1.6% copper, 0.4% cobalt, 40.0% iron, 31.0% sulfur and 7% silica. This concentrate was autogenously smelted with oxygen to a matte containing 48.2% nickel, 8.6% copper, 1.6% cobalt, 28% sulfur and the balance mainly iron. 55 The slag from this operation containing 1.5% nickel was removed for separate treatment to recover its metal values. The matte was then blown with oxygen to produce a substantially iron-free matte which was tapped to leave a high nickel slag in the furnace for subsequent reduction with fresh charge. This matte was treated for copper removal at 1400° F. by our solvent extraction technique as described hereinbefore in Example III. The resulting substantially iron- and copper-free matte was treated to remove cobalt by the process described in Example IV. 60 65 70 75 The thus-treated matte was top blown with oxygen at a temperature rising to 2850° F. to a sulfur content of 3%. The thus blown matte can then be treated, as has been described above, for final sulfur elimination.

#### EXAMPLE VI

75 4.4 tons of a molten nickel matte containing 70.9% nickel, 4.8% copper, 1.0% iron and 23.3% sulfur were top blown with oxygen in a furnace, similar to that shown in FIGURE 2, rotating at 20 r.p.m. at a temperature rising to 3000° F. Cooling was accomplished by in-

jecting air with the oxygen. The molten material was blown down to 1.4% sulfur at which point propane gas was injected with the oxygen and rotation of the furnace was increased to 30 r.p.m. Enough propane was injected to produce a somewhat reducing atmosphere in the furnace. The temperature of the bath rose to and was held at about 3100° F. and the molten bath was blown to a sulfur content of 0.02%. The bath at the end of the blow had an oxygen content of 1.9% which was removed by adding graphite to the bath in the furnace. Total blowing time to final desulfurization was seven hours and fifty minutes.

#### EXAMPLE VII

To illustrate the extreme importance of strong mechanically induced agitation of the molten bath during blowing, 4.3 tons of the same nickel matte as treated in Example VI were blown with oxygen in a manner similar to that used in these examples except that the furnace remained stationary. After eight hours and forty minutes of blowing the sulfur content of the metal had been decreased to only 2%, further reaction ceased and blowing had to be discontinued because of nickel oxide accumulation with formation of a heavy impenetrable layer of slag floating on the metal.

It is to be observed that by the above described invention, metallic nickel can be produced directly from nickel concentrates obtained by flotation of nickel sulfide ores after copper removal by our novel techniques as described hereinbefore. It is known that pentlandite concentrate may be oxygen-flash smelted to a nickel matte, as disclosed by one of the present inventors in U.S. Patent No. 2,668,107. Our new process is an improvement over that described in this patent in that our product is metallic nickel instead of nickel matte with a high impurities content. Summarizing our technique for treating nickel concentrates by our novel process to obtain metallic nickel directly, we charge dry nickel concentrate, e.g., pentlandite concentrate, into molten material in an autogenous reduction furnace, such as described hereinbefore, and blow for removal of iron which may be slagged off by addition of siliceous flux. The slag produced during the first stage of iron elimination, low in nickel, is removed from the furnace and the slag produced during the final stage of iron elimination is left in the furnace for extraction of its nickel content upon further addition of concentrate. After iron removal is completed, the molten material may be treated for copper removal and it is then blown directly to metallic nickel both of which operations are above described in detail.

It is further to be observed that the herein-described process is highly suitable for the treatment of crude mattes obtained from lateritic nickel-containing ores as for instance, by the process described by one of the present inventors in the copending U.S. patent application Serial No. 51,418, filed August 23, 1960, now U.S. Patent 3,004,846. These mattes which contain substantial amounts of iron and some cobalt can be blown in the autogenous reduction furnace for iron, sulfur and cobalt removal and direct production of metallic nickel. Since these lateritic ores normally contain substantially no copper or precious metals, the molten material need not be treated for their removal but in the case of ores with a substantial cobalt content, the matte may be treated for cobalt removal as described herein.

It is to be observed also that prior art techniques for directly reducing nickel-rich matte to commercial metallic nickel or nickel-copper alloys failed utterly because of formation of metal oxides rather than metal with resultant massive accumulations of accretions and of floating dross which smothered the reaction long before it was complete and also because of destruction of refractories due to subsurface blowing of the bath and/or lack of proper bath turbulence with consequent excessive local temperature rise.

Furthermore, it is to be observed that our novel copper removal technique, by high temperature liquid-liquid separation is a major advance over the now long obsolete Orford process which was abandoned because of its high cost and the low separation efficiency of its batch-type operation.

This application is a continuation-in-part of our copending U.S. application Serial No. 839,431, filed September 11, 1959, now abandoned.

10 Although the present invention has been described in conjunction with preferred embodiments, it is to be understood that modifications and variations may be resorted to without departing from the spirit and scope of the invention, as those skilled in the art will readily understand. Thus, our process may be employed for the treatment of copper-rich materials, e.g., copper flotation concentrates and mattes to yield directly fire-refined or anode copper. Such modifications and variations are considered to be within the purview and scope of the 15 invention and appended claims.

We claim:

1. An improved process for autogenously converting a nickel sulfide material to produce nickel of low sulfur content which comprises directing oxidizing gases from 20 the group consisting of commercial oxygen and oxygen-enriched air into the exposed surface of a molten bath of said sulfide material, while avoiding sidewall and bottom blowing of said gases through the bath, and maintaining the bath during the converting in a state of 25 turbulence with non-pneumatic, mechanically induced agitation, said agitation being maintained during the directing of said oxidizing gases, to promote intimate and efficient gas-liquid-solid contact and uniform distribution of oxygen throughout the bath and its rapid reaction with 30 sulfur therein; raising the bath temperature as desulfurization proceeds to more than about 2800° F.; changing said gases being introduced into the bath surface to hot, substantially sulfur-free gases from the group 35 consisting of neutral and reducing gases having an oxygen content insufficient to cause visible formation of 40 interfering amounts of nickel oxide dross on the surface of the bath when the sulfur content of the bath is still substantial but is less than about 4% and the oxygen content of the bath is at least sufficient to oxidize the sulfur content, the bath being at a temperature of at 45 least about 3000° F. and maintained in a turbulent state by non-pneumatic, induced agitation upon changing from oxygen-rich gases; and maintaining a bath temperature of at least about 3000° F. in the presence of 50 said hot gases to continue the reaction between sulfur and oxygen in the turbulent bath and to produce nickel with a sulfur content low enough below 0.5% for removal by desulfurization.

2. A process as described in claim 1 in which mechanically induced agitation of the molten bath is attained by rotation of the furnace and the metallic nickel obtained contains not more than about 0.02% sulfur.

3. An improved process for autogenously converting a nickel sulfide material to produce refined nickel of low sulfur content which comprises blowing commercial oxygen onto the exposed surface of a molten bath of said sulfide material while avoiding sidewall and bottom blowing of said oxygen through the bath, and maintaining the bath substantially slag free during the blowing with oxygen and in a state of turbulence with mechanically induced agitation, said agitation being maintained during the blowing, to promote intimate and efficient gas-liquid-solid contact and uniform distribution of oxygen throughout the bath and its rapid reaction with sulfur therein and to produce off-gas rich in sulfur dioxide; raising the bath temperature as desulfurization proceeds to more than about 2800° F. while continuing said blowing with oxygen; transferring the bath to a substantially sulfide-free furnace environment when the 70 sulfur content of said bath is still substantial but is less 75

than about 4% and its oxygen content is at least sufficient to oxidize the sulfur content; blowing onto said transferred bath, maintained in a state of turbulence by mechanically induced agitation, hot gases from the group consisting of neutral and reducing gases substantially free of sulfur dioxide and having an oxygen content insufficient to cause visible formation of interfering amounts of nickel oxide dross on the surface of the bath, the transferred bath being at a temperature of at least about 3000° F.; maintaining a bath temperature of at least about 3000° F. in the presence of said hot gases to continue the reaction between sulfur and oxygen in the turbulent bath and to obtain metallic nickel; and de-oxidizing the molten bath to produce refined nickel with a low sulfur content of not more than of the order of about 0.05%.

4. In a process for producing refined, metallic nickel from nickel-rich sulfide materials containing iron in which the sulfide material is smelted to produce a nickel-iron matte and the nickel-iron matte is blown to remove iron therefrom and form a nickel matte, the improvement which comprises autogenously smelting the nickel matte by blowing commercial oxygen onto the exposed surface of a molten bath of said nickel matte at a temperature of at least about 2400° F., while avoiding sidewall and bottom blowing of said oxygen through the bath, and maintaining the bath substantially free of slag during the blowing with oxygen and in a state of turbulence with mechanically induced agitation, said agitation being maintained during the blowing to promote intimate and efficient gas-liquid-solid contact and uniform distribution of oxygen throughout the bath and its rapid reaction with sulfur therein; raising the bath temperature as desulfurization proceeds to more than about 2800° F. while continuing said blowing with oxygen; changing said oxygen being directed onto the molten bath to hot gases from the group consisting of neutral and reducing gases substantially free of sulfur dioxide and having an oxygen content insufficient to cause visible formation of interfering amounts of nickel oxide dross on the surface of the bath when its sulfur content is between about 1% and about 3% and its oxygen content is at least sufficient to oxidize the sulfur content, the bath being at a temperature of between about 3000° F. and 3200° F. and maintained in a turbulent state by mechanically induced agitation upon changing from oxygen; and maintaining a bath temperature of between about 3000° F. and 3200° F. in the presence of said hot gases to continue the reaction between sulfur and oxygen in the turbulent bath and to produce refined, pig nickel with a low sulfur content of not more than of the order of about 0.05%.

5. An autogenous process for producing refined metallic nickel directly from nickel-rich sulfide materials containing iron which comprises directing commercial oxygen onto the surface of a molten bath of said nickel-rich sulfide material while avoiding sidewall and bottom blowing of said oxygen through the bath, said bath being maintained in a state of turbulence by mechanically induced agitation, said agitation being maintained during the directing of said oxygen, to oxidize iron and desulfurize the bath; slagging the oxidized iron with silica flux and drawing off the slag so formed; raising the temperature of the molten bath after slagging of said iron and as desulfurization proceeds to attain a bath temperature of at least about 2800° F., while continuing the directing of oxygen onto the molten bath maintained in a state of induced turbulence to promote intimate and efficient gas-liquid-solid contact and uniform distribution of oxygen throughout the bath and its rapid reaction with sulfur therein; changing said oxygen being directed onto the molten bath to hot gases from the group consisting of neutral and reducing gases substantially free of sulfur dioxide and having an oxygen content insufficient to cause visible formation of interfering

5  
10  
15  
20  
25  
30  
35  
40  
45  
50  
55  
60  
65  
70  
75

amounts of nickel oxide dross on the surface of the bath when its sulfur content is between about 1% and about 3% and its oxygen content is at least sufficient to oxidize the sulfur content, the bath being at a temperature of at least about 3000° F. and maintained in a turbulent state by mechanically induced agitation upon changing from oxygen; and maintaining a bath temperature of at least about 3000° F. in the presence of said hot gases to continue the reaction between sulfur and oxygen in the turbulent bath and to produce refined, pig nickel with a low sulfur content of not more than of the order of about 0.05%.

6. A process as described in claim 5 in which the nickel-rich sulfide material contains cobalt and wherein, after iron is oxidized, slagged and drawn off, the sulfur content of the metal bath is maintained at greater than about 3% by adding fresh sulfide material while blowing with oxygen at between about 2300° F. and about 2800° F. to oxidize the cobalt and remove it as slag.

7. An improved process for autogenously converting a nickel-copper sulfide material to produce nickel-copper-alloy of low sulfur content which comprises directing oxygen-rich gases from the group consisting of commercial oxygen and oxygen-enriched air into the exposed surface of a molten bath of said sulfide material, while avoiding sidewall and bottom blowing of said gases through the bath, and maintaining the bath during the converting in a state of turbulence with non-pneumatic, mechanically induced agitation, said agitation being maintained during the directing of said oxygen-rich gases, to promote intimate and efficient gas-liquid-solid contact and uniform distribution of oxygen throughout the bath and its rapid reaction with sulfur therein; raising the bath temperature as desulfurization proceeds while maintaining its surface substantially free of oxide dross; changing said gases being introduced into the bath surface to hot, substantially sulfur-free gases from the group consisting of neutral and reducing gases having an oxygen content insufficient to cause visible formation of interfering amounts of nickel oxide dross on the surface of the bath when its sulfur content is still substantial but is less than about 4% and its oxygen content is at least sufficient to oxidize the sulfur content, the bath being maintained in a turbulent state by non-pneumatic, induced agitation and at a high temperature sufficient to minimize the formation of oxide dross on the surface of the nickel-copper alloy bath upon changing from oxygen-rich gases; and maintaining the high temperature in the bath in the presence of said hot gases to continue the reaction between sulfur and oxygen in the turbulent bath and to produce nickel-copper alloy with a sulfur content low enough below 0.5% for removal by desulfurization.

8. An improved process for eliminating copper from and autogenously smelting a nickel sulfide material containing copper to produce refined, pig nickel of low sulfur content which comprises melting and mixing between about one-half to double by weight of a mixture of sodium chloride and sodium sulfide salts with said nickel sulfide material in the molten state; allowing said molten mass to separate into an upper copper-rich and sodium salt-containing liquid phase and a lower nickel sulfide liquid phase; separating said liquid phases; treating said upper liquid phase for recovery of the sodium salts contained therein; oxidizing and removing sodium salts from the lower, nickel sulfide liquid phase; directing oxygen onto the exposed surface of a molten bath of said nickel sulfide phase, while avoiding sidewall and bottom blowing of said oxygen through the bath, and maintaining the bath during the smelting in a state of turbulence with mechanically induced agitation, said agitation being maintained during the directing of said oxygen, to promote intimate and efficient gas-liquid-solid contact and uniform distribution of oxygen throughout the bath and its rapid reaction with sulfur therein; raising the bath temperature

as desulfurization proceeds to more than about 2800° F. while continuing the directing of oxygen onto the bath; changing said oxygen being directed onto the molten bath to hot gases from the group consisting of neutral and reducing gases substantially free of sulfur dioxide and having an oxygen content insufficient to cause visible formation of interfering amounts of nickel oxide dross on the surface of the bath when its sulfur content is between about 1% and about 3% and its oxygen content is at least sufficient to oxidize the sulfur content, the bath being at a temperature of at least about 3000° F. and maintained in a turbulent state by mechanically induced agitation upon said changing from oxygen; and maintaining a bath temperature of at least about 3000° F. in the presence of said hot gases to continue the reaction between sulfur and oxygen in the turbulent bath and to produce refined, pig nickel with a low sulfur content of not more than of the order of about 0.05%.

9. In the treatment of a nickel sulfide material with a copper content of at least about 0.50% for elimination of the copper and recovery of the nickel contained therein, the improvement which comprises melting and mixing between about one-half to double by weight of a salt mixture of sodium sulfide and a metal chloride from the group consisting of sodium chloride, potassium chloride, calcium chloride and aluminum chloride with said nickel sulfide material in the molten state; allowing said molten mass to separate into an upper copper sulfide-salt mixture liquid phase and a lower nickel sulfide liquid phase; separating said liquid phases; treating said upper liquid phase for recovery of the salt mixture contained therein; oxidizing and removing salt mixture from the lower, nickel sulfide liquid phase; and treating said nickel sulfide liquid phase for recovery of the nickel contained therein.

10. A process as described in claim 9 in which the salt mixture is sodium chloride and sodium sulfide and contains between about 25% and about 75% sodium chloride, the separation of the copper sulfide-salt mixture phase and the nickel sulfide phase is carried out in a liquid-liquid extraction column and the nickel sulfide phase separated out contains less than 0.10% copper.

11. In the treatment of a nickel sulfide material with a copper content of at least about 0.50% for elimination of the copper and recovery of the nickel contained therein, the improvement which comprises melting and mixing between about one-half to double by weight of a mixture of sodium chloride and sodium sulfide salts containing between about 25% and about 75% sodium chloride with said nickel sulfide material in the molten state at a temperature of not below about 1350° F. and not above about 1550° F.; allowing said molten mass to separate into an upper copper sulfide and sodium salt-containing liquid phase and a lower nickel sulfide liquid phase with a copper content of less than about 0.10%; separating said upper and lower phases by pouring one from the other in the liquid state; treating said upper liquid phase for recovery of the sodium salts contained therein; reverting said sodium salts for further copper elimination; oxidizing and removing any sodium salts from the lower, nickel sulfide liquid phase; and treating the nickel sulfide remaining for recovery of the nickel contained therein.

12. In the treatment of cobalt-containing nickel sul-

fide material with a copper content of at least about 0.50% for elimination of the copper and cobalt and recovery of the nickel contained therein as refined, pig nickel of low sulfur content, the improvement which comprises melting and mixing between about one-half to double by weight of a salt mixture of sodium sulfide and a metal chloride from the group consisting of the chlorides of sodium, potassium, calcium and aluminum with said nickel sulfide material in the molten state; allowing said molten mass to separate into an upper copper sulfide-salt mixture liquid phase and a lower nickel sulfide liquid phase; repeating the foregoing operations in a countercurrent manner; separating the final liquid phases; treating the upper liquid phase for recovery of the copper and the salt mixture contained therein; oxidizing and removing salt mixture from the final, lower, nickel sulfide liquid phase; directing commercial oxygen onto the exposed surface of a molten bath of said nickel sulfide from which copper has been eliminated, while avoiding sidewall and bottom blowing of said oxygen through the bath, and maintaining the bath in a state of turbulence by mechanically induced agitation, said agitation being maintained during the directing of said oxygen, to promote intimate and efficient gas-liquid-solid contact and uniform distribution of oxygen throughout the bath and its rapid reaction with sulfur therein; maintaining the sulfur content of the molten bath at more than about 3% by adding substantially copper-free fresh nickel sulfide material, while blowing with oxygen at between about 2300° F. and about 2800° F. to oxidize the cobalt and remove it as slag; raising the temperature of the molten bath when cobalt has been eliminated and slagged off and as desulfurization proceeds to more than about 2800° F. while continuing the directing of oxygen onto the bath; changing said oxygen being directed onto the molten bath to hot gases from the group consisting of neutral and reducing gases substantially free of sulphur dioxide and having an oxygen content insufficient to cause visible formation of interfering amounts of nickel oxide dross on the surface of the bath when its sulfur content is still substantial but is less than about 4% and its oxygen content is at least sufficient to oxidize the sulfur content, the bath being at a temperature of between about 3000° F. and 3200° F. and maintained in a turbulent state by mechanically induced agitation upon said changing from oxygen; and maintaining a bath temperature of between about 3000° F. and 3200° F. in the presence of said hot gases to continue the reaction between sulfur and oxygen in the turbulent bath and to produce refined, pig nickel with a low sulfur content of not more than of the order of about 0.05%.

#### References Cited in the file of this patent

#### UNITED STATES PATENTS

|    |           |                |                |
|----|-----------|----------------|----------------|
| 55 | 1,599,424 | Lellep         | Sept. 14, 1926 |
|    | 1,623,797 | Lellep         | Apr. 5, 1927   |
|    | 1,703,329 | Wilenchik      | Feb. 26, 1929  |
|    | 1,877,928 | McGregor       | Sept. 20, 1932 |
| 60 | 2,396,792 | Kroll          | Mar. 19, 1946  |
|    | 2,598,393 | Kalling et al. | May 27, 1952   |
|    | 2,653,868 | Lichty         | Sept. 29, 1953 |